

## 1

2,996,454

**METHOD OF PROTECTING MACHINERY FROM CORROSION BY ACID-REACTING SUBSTANCES TENDING TO ACCUMULATE IN LUBRICATING OILS**

Abraham Shapiro, Los Angeles, Calif., assignor to Socony Mobil Oil Company, Inc., New York, N.Y., a corporation of New York  
No Drawing. Filed July 7, 1958, Ser. No. 746,675  
4 Claims. (Cl. 252—50)

This invention relates to protection of engines and other machinery from the corrosive effects of acid-reacting substances which tend to accumulate in lubricating oils.

The problem is a familiar one in internal-combustion engines which employ fuels of high sulfur content. Sulfur dioxide and other acidic oxidation products are produced in the cylinders, and some of the acidic material finds its way into the crankcase oil with the result that bearings and other parts are exposed to corrosion.

Various oil-soluble basic substances have been added to lubricating oils for the purpose (among others) of neutralizing acid-reacting substances which tend to contaminate the oils. These have functioned satisfactorily when the quantity of acid material is small, as in gasoline engines employing fuels of low sulfur content. But when highly sulfurous fuels are used, any reasonable amount of basic additive in the lubricating oil becomes neutralized and ineffective long before the oil is otherwise ready for replacement.

Another procedure, common in marine usage, has been to periodically or continuously remove oil from the crankcase, agitate it with water, separate the oil from the water in a centrifuge, and return the washed oil to the crankcase. This method prevents the oil from becoming more than mildly corrosive but it does not completely prevent corrosion.

Heretofore, these two procedures have been incompatible with one another. The oil-soluble basic substances which have been added to lubricating oils, or their sulfites and similar salts, have acted as emulsifying agents. Consequently, when oils containing them have been agitated with water, emulsions have formed which cannot be separated by centrifugal treatment or other methods practical for use by operators of engines. For this reason it has been customary to omit basic additives from lubricating oils which are to be washed with water.

I have discovered that the two procedures can be combined if a particular basic material or its components are employed in a lubricating oil. The material is the fraction of nitrogen bases from coal tar having a boiling range of 240° to 265° C. This fraction is soluble in oil and insoluble in water, it is adequately stable with respect to oxidation, it combines with sulfur dioxide and other corrosive acid substances to form salts which are soluble in water and have only limited solubility in oil, and it has no tendency to stabilize emulsions of lubricating oil and water. It is, therefore, extremely effective in neutralizing corrosive substances and transferring them from the oil to the wash water.

It is necessary to exclude from the lubricating oil the nitrogen bases which act as emulsifying agents or which are subject to oxidation or other chemical changes whereby emulsifying agents or gummy substances are formed.

The above-described material, employed as an additive for lubricating oils, also provides a solution for problems encountered with oils which are not intentionally washed with water but which are subject to being brought into contact with water in other ways. For example, crankcase oils may be contaminated with water which con-

## 2

denses from the combustion products or by water which leaks from the cooling systems of engines. The previously employed basic additives have caused this water to emulsify with the oil. The additive herein disclosed allows the accidentally introduced water to separate from the oil, thus permitting continued use of oil which otherwise would require early replacement.

The fraction consists essentially of the methylquinolines, the methyliisoquinolines, and isoquinoline. The various members of this group of chemical compounds and their mixtures are all capable of serving the purposes set forth herein. But quinoline itself, being a water-soluble substance, is not suitable for use.

In the processing of coal tar it is usual to treat the tar or a distillate fraction of it with dilute sulfuric acid to extract basic constituents, to free the bases from the resulting aqueous solution by addition of caustic soda or other alkali, and to distill the mixture of free bases to obtain products such as quinoline. The separation of quinoline in this manner yields as a by-product a distillation residue having an initial boiling point of about 240° C.

This residue consists mainly of methylquinolines, methyliisoquinolines, and isoquinoline but, in the form available in commerce, it also contains tarry substances which make it unsuitable for use as an additive for lubricating oils. By subjecting the commercially available residue to vacuum distillation at a pressure of not more than about 0.1 atmosphere to produce an overhead fraction with a boiling range of 240° to 265° C. and discarding the still base (which amounts to about 10% of the original material), a substance fully satisfactory for blending with lubricating oil is obtained.

By parallel procedure nitrogen-base fractions can be prepared from petroleum distillates, but these are complex, malodorous mixtures that are rich in constituents which oxidize readily to produce gummy substances. Therefore the nitrogen bases from petroleum are not desirable for the purposes set forth herein.

Small amounts of the additive herein disclosed do not adversely affect any of the desired properties of lubricating oils. As the proportion of additive is increased, the first lubricating-oil property to suffer is the flash point. Use of 4% of the additive brings the flash point of ordinary lubricants down to about 350° F. (Cleveland open cup), which is the minimum most often specified for crankcase oils. The additive also tends to decrease the viscosity of an oil, at least as measured at 100° F., but this can be readily counteracted by use of a more viscous lubricant stock.

If desired, the tendency of the material to depress flash points of oils can be ameliorated by distilling off the more volatile components and using the less volatile portion as the additive. The more volatile portion, consisting mainly of isoquinoline or of a mixture of isoquinoline and quinaldine, need not be discarded but can be used in oils in which lower flash points are permissible or in which lesser amounts of the additive are needed. I have found that, merely by heating the material in an open container to temperatures of 450° to 500° F. until the volume is reduced to 90% of the original, the flash points of oils compounded with 4% of additive are increased by about 20° F.

By reducing the volatility of the additive it is possible to compound oils having considerably more than 4% of the additive even when a minimum flash point of 350° F. is specified. When the flash point is not a critical property no definite maximum for the proportion of additive can be stated, for very large amounts can be used without diminishing viscosity and lubricity to the points where an oil ceases to be useful as a lubricant. In oils which are used in severely acid conditions without periodic

washing, the prolongation of the period of protection from acid may more than compensate for a moderate sacrifice of lubricant properties.

If plain water or sea water is used to wash the oil, the neutralized nitrogen bases are removed from the oil and discarded with the water. Consequently, the proportion of additive in the oil keeps diminishing. It continues to protect bearings and other parts from corrosion until it falls below about 0.1%, but when that occurs more of the additive should be put in the oil.

Operators of engines cannot be expected to have facilities for determining the percentage of nitrogen bases in an oil, but an operator with a normal olfactory sense can make a rough but adequate determination by smelling the washed and separated oil; if the characteristics quinoline-like odor is absent or very weak, the content of additive in the oil should be replenished. Another method is to shake the used, unwashed oil with distilled water and to test the water with litmus, and to replenish the additive in the washed and separated oil if an acid reaction is noted. The latter test does not necessarily indicate the presence or absence of nitrogen bases, but it can be assumed that an oil which does not test acid with litmus is substantially noncorrosive either because of low concentration of acidic substances or because of the presence of enough basic material to effect adequate neutralization.

Maintenance of a sufficient quantity of the additive in an oil can also be achieved, in most cases more economically, by employing wash water which has been alkalinized by addition of up to 1.0% of caustic soda or its equivalent. When this is done the alkaline water decomposes the salts of the nitrogen bases, and the free bases (being oil-soluble and water-insoluble) return to the lubricating oil and continue to protect metallic parts from corrosion. I have found that when oils containing the herein-described additive are saturated with sulfur dioxide, agitated with alkaline water, and separated from the water by centrifugal treatment, the washed oils are indistinguishable with regard to pH and other properties from the same oils which had not been exposed to sulfur dioxide.

The table shows representative properties of four different mineral lubricating-oil stocks and, as specific examples of lubricants compounded according to this invention, oils prepared from those stocks by addition of 1% and 4% of the fraction of coal-tar nitrogen bases having a boiling range of 240° to 265° C. In the table proportions of the additive are expressed as percentages by weight with respect to the total oil, flash points and pour points are in degrees Fahrenheit, and viscosities are in seconds Saybolt Universal.

|                    | Stock A |      |       | Stock B |      |      | Stock C |       |       | Stock D |       |       |
|--------------------|---------|------|-------|---------|------|------|---------|-------|-------|---------|-------|-------|
| Percent additive   | 0       | 1    | 4     | 0       | 1    | 4    | 0       | 1     | 4     | 0       | 1     | 4     |
| Gravity, A.P.I.    | 26.8    | 27.2 | 25.2  | 26.4    | 26.4 | 25.0 | 25.9    | 25.7  | 24.3  | 25.0    | 25.0  | 23.7  |
| Color, A.S.T.M.    | L4.5    | L6   | 7     | L5      | D7   | L8   | 7       | D7    | 8     | 7       | L8    | D8    |
| Flash, C.O.C.      | 425     | 395  | 340   | 440     | 395  | 340  | 460     | 400   | 345   | 480     | 410   | 355   |
| Pour point         | -10     | +15  | +15   | -5      | +15  | +15  | +15     | +15   | +10   | +15     | +15   | +5    |
| Visc. @ 100° F.    | 530     | 493  | 475   | 942     | 844  | 832  | 1,329   | 1,299 | 1,297 | 1,986   | 1,927 | 1,902 |
| Visc. @ 210° F.    | 61.7    | 62.0 | 61.4  | 76.0    | 77.9 | 77.2 | 93.9    | 96.2  | 96.0  | 117.0   | 118.9 | 117.5 |
| Visc. index        | 82      | 92   | 93    | 69      | 88   | 87   | 79      | 86    | 86    | 80      | 85    | 84    |
| Neutralization No. | .01     | .03  | .02   | .01     | .03  | .03  | .01     | .03   | .03   | .01     | .03   | .05   |
| Carbon residue     | .15     | .21  | .23   | .24     | .25  | .31  | .35     | .35   | .42   | .69     | .37   | .49   |
| pH                 | 8.1     | 8.2  | ----- | 8.1     | 8.4  | 6.2  | 8.0     | 8.5   | ----- | 8.0     | 8.7   | ----- |
| Total base No.     | 0.18    | 0.8  | ----- | 0.21    | 0.7  | 0.04 | 0.24    | 1.0   | ----- | 0.15    | 0.7   | ----- |

In addition to the properties reported in the table, corrosion tests were run on Stock C and the compounded oils prepared from it, by immersing polished metal strips in the oils for twenty-four hours at a temperature of 150° F. The steel and aluminum strips showed no change in any of the oils. Copper, however, was tarnished by the oil which contained no additive and was left bright by the oils which did contain the additive.

Another specific example of the lubricating oils of the

present invention was compounded with 1% of the fraction of coal-tar bases having a boiling range of 240° to 265° C. and 99% of a mineral lubricating oil having viscosities of 1275 and 101 S.S.U at 100° F. and 210° F. respectively and a pH of 4.7. The resulting composition had viscosities of 929 and 85.8 at 100° F. and 210° F. respectively and a pH of 5.5. This example was used in a 6-cylinder Buda engine employing as fuel a gasoline of 0.65% sulfur content for a test run of 200 hours. The test indicated that use of the additive had no observable effect upon lubricity of the oil, that it did not lead to formation of undesirable deposits on metallic parts, and that it was successful in neutralizing acid oxidation products under actual operating conditions.

- 15 I claim as my invention:
1. In a method of protecting machinery from corrosion by acid-reacting substances tending to accumulate in the oil employed to lubricate said machinery which includes washing said oil by agitation with an aqueous liquid, separating the washed oil from said aqueous liquid, and returning the washed and separated oil to said machinery, the improvement which comprises: maintaining in said oil at least 0.1 percent by weight of a mixture of organic basic substances derived by extracting bases from coal tar with an aqueous acid solution, subsequently alkalinizing said solution to free organic bases therefrom, and distilling the free bases to obtain a fraction having an initial boiling point of at least 240° C. and an end point of 265° C.
  - 20 2. A method as described in claim 1, wherein said aqueous liquid is approximately neutral and said quantity of said basic material is maintained in said oil by periodic addition of further amounts of said material to said oil.
  - 25 3. A method as described in claim 1, wherein said quantity of said basic material is maintained in said oil by making said aqueous liquid sufficiently alkaline to decompose salts of said basic material but not more alkaline than a one-percent aqueous solution of caustic soda.
  - 30 4. In a method of protecting machinery from corrosion by acid-reacting substances tending to accumulate in the oil employed to lubricate said machinery which includes washing said oil by agitation with an aqueous liquid, separating the washed oil from said aqueous liquid, and returning the washed and separated oil to said machinery, the improvement which comprises: maintaining in said oil at least 0.1 percent by weight of a mixture of organic basic substances derived by extracting bases from coal tar with an aqueous acid solution, subsequently alkalinizing said solution to free organic bases therefrom, and
  - 35 5. A method as described in claim 1, wherein said quantity of said basic material is maintained in said oil by making said aqueous liquid sufficiently alkaline to decompose salts of said basic material but not more alkaline than a one-percent aqueous solution of caustic soda.
  - 40 6. In a method of protecting machinery from corrosion by acid-reacting substances tending to accumulate in the oil employed to lubricate said machinery which includes washing said oil by agitation with an aqueous liquid, separating the washed oil from said aqueous liquid, and returning the washed and separated oil to said machinery, the improvement which comprises: maintaining in said oil at least 0.1 percent by weight of a mixture of organic basic substances derived by extracting bases from coal tar with an aqueous acid solution, subsequently alkalinizing said solution to free organic bases therefrom, and
  - 45 7. A method as described in claim 1, wherein said quantity of said basic material is maintained in said oil by making said aqueous liquid sufficiently alkaline to decompose salts of said basic material but not more alkaline than a one-percent aqueous solution of caustic soda.
  - 50 8. In a method of protecting machinery from corrosion by acid-reacting substances tending to accumulate in the oil employed to lubricate said machinery which includes washing said oil by agitation with an aqueous liquid, separating the washed oil from said aqueous liquid, and returning the washed and separated oil to said machinery, the improvement which comprises: maintaining in said oil at least 0.1 percent by weight of a mixture of organic basic substances derived by extracting bases from coal tar with an aqueous acid solution, subsequently alkalinizing said solution to free organic bases therefrom, and

65 distilling the free bases to obtain a fraction having a boiling range of 240° C. to 165° C.

#### References Cited in the file of this patent

#### UNITED STATES PATENTS

- 70 1,768,910 Ihrig ----- July 1, 1930  
 2,136,788 Fairlie ----- Nov. 15, 1938  
 2,441,849 Sexton et al. ----- May 18, 1948  
 2,647,824 Jones et al. ----- Aug. 4, 1953

UNITED STATES PATENT OFFICE  
CERTIFICATE OF CORRECTION

Patent No. 2,996,454

August 15, 1961

Abraham Shapiro

It is hereby certified that error appears in the above numbered patent requiring correction and that the said Letters Patent should read as corrected below.

Column 3, line 12, for "is" read -- in --; line 15, for "characteristics" read -- characteristic --; line 35, for "he" read -- the --; column 4, line 5, for "repectively" read -- respectively --; line 66, for "165° C." read -- 265° C. --.

Signed and sealed this 27th day of March 1962.

(SEAL)

Attest:

ERNEST W. SWIDER

Attesting Officer

DAVID L. LADD

Commissioner of Patents

UNITED STATES PATENT OFFICE  
CERTIFICATE OF CORRECTION

Patent No. 2,996,454

August 15, 1961

Abraham Shapiro

It is hereby certified that error appears in the above numbered patent requiring correction and that the said Letters Patent should read as corrected below.

Column 3, line 12, for "is" read -- in --; line 15, for "characteristics" read -- characteristic --; line 35, for "he" read -- the --; column 4, line 5, for "repectively" read -- respectively --; line 66, for "165° C." read -- 265° C. --.

Signed and sealed this 27th day of March 1962.

(SEAL)

Attest:

ERNEST W. SWIDER

Attesting Officer

DAVID L. LADD  
Commissioner of Patents